

## UNITED STATES PATENT OFFICE

1,928,382

## PERMANENT MAGNET

Werner Köster, Dortmund, Germany, assignor  
to Vereinigte Stahlwerke Aktiengesellschaft,  
Dusseldorf, Germany

No Drawing. Application May 12, 1931, Serial  
No. 536,950, and in Germany May 23, 1930

3 Claims. (Cl. 175—21)

This invention relates to permanent magnets  
resistant to changes of temperature.

The magnets hitherto manufactured by hardening  
a relatively high carbon steel are not resistant  
5 to temperature changes or annealing. The mar-  
tensitic structure which they exhibit and which  
is the cause of their magnetic values gradually  
changes even at lower temperatures. At the  
same time the magnetic hardness constantly de-  
10 creases. If therefore such a magnet be built  
into an apparatus which operates at elevated  
temperatures then on cooling to lower tempera-  
tures, for example, room temperature, the said  
magnet does not revert to its original state.  
15 The present invention obviates the foregoing  
drawback and relates to a permanent magnet  
which is resistant to temperature changes due to  
its manufacture from a special kind of ferro-  
magnetic alloy which is adapted to be age-  
20 hardened, that is to say, which can be improved  
by a precipitation hardening and which is after  
such precipitation hardening stable against the  
high temperatures to which it had been subjected  
during the annealing treatment causing the pre-  
25 cipitation hardening. These alloys are first  
quenched for the purpose of attaining their high-  
est magnetic properties, and then annealed at  
elevated temperatures (up to about 700° C.). In  
consequence of this heat treatment they are  
30 completely stable to temperature changes up to  
the previous annealing temperature. After heat-  
ing to elevated temperatures they revert to their  
initial values on cooling. This property is fre-  
quently very desirable in the construction of  
35 machines, apparatus and measuring instruments.  
It could however, up to the present, not be at-

tained with the magnetic alloys hitherto usual.  
Such requirements are for example, made in the  
construction of temperature regulators, contacts,  
measuring instruments and the like.

By way of example an alloy may be mentioned, 30  
the main constituents of which are 15 per cent of  
tungsten and 30 per cent of cobalt, the remainder  
being iron. If such an alloy be quenched from  
1200° C. and be annealed for one hour at 700° C.  
there is thus obtained a coercive force of about 65  
85 gausses. The alloy thus treated can now be  
heated, to a temperature of about 700° C. with-  
out its magnetic hardness being decreased there-  
by. This process is generally known as "age  
hardening" or precipitation hardening. 70

I claim:—

1. A permanent magnet resistant to tempera-  
ture changes which comprises a ferromagnetic  
alloy magnetically stable against temperature  
changes up to about 700° C. 75

2. A permanent magnet resistant to tempera-  
ture changes which comprises a ferromagnetic  
alloy subjected to precipitation hardening, con-  
taining as main constituents, 15 per cent of  
tungsten and 30 per cent of cobalt and the re- 80  
mainder iron.

3. A method of preparing an alloy for perma-  
nent magnets, which consists in precipitation  
hardening of a ferromagnetic alloy by first  
quenching said alloy from a temperature of about 85  
1200° C. for the purpose of obtaining its highest  
magnetic properties, and then annealing the alloy  
at temperatures up to 700° C., said alloy contain-  
ing as main constituents approximately 15%  
tungsten, 30% cobalt and the remainder iron. 90

WERNER KÖSTER.

## DISCLAIMER

1,928,382.—Werner Köster, Dortmund, Germany. PERMANENT MAGNET. Patent  
dated September 26, 1933. Disclaimer filed August 2, 1938, by the assignee,  
Deutsche Edelstahlwerke A. G.

Hereby enters this disclaimer to claim 1 in said specification.  
[Official Gazette September 6, 1938.]

## UNITED STATES PATENT OFFICE

1,928,382

## PERMANENT MAGNET

Werner Köster, Dortmund, Germany, assignor  
to Vereinigte Stahlwerke Aktiengesellschaft,  
Dusseldorf, Germany

No Drawing. Application May 12, 1931, Serial  
No. 536,950, and in Germany May 23, 1930

3 Claims. (Cl. 175—21)

This invention relates to permanent magnets  
resistant to changes of temperature.

The magnets hitherto manufactured by hardening  
a relatively high carbon steel are not resistant  
5 to temperature changes or annealing. The mar-  
tensitic structure which they exhibit and which  
is the cause of their magnetic values gradually  
changes even at lower temperatures. At the  
same time the magnetic hardness constantly de-  
10 creases. If therefore such a magnet be built  
into an apparatus which operates at elevated  
temperatures then on cooling to lower tempera-  
tures, for example, room temperature, the said  
magnet does not revert to its original state.  
15 The present invention obviates the foregoing  
drawback and relates to a permanent magnet  
which is resistant to temperature changes due to  
its manufacture from a special kind of ferro-  
magnetic alloy which is adapted to be age-  
20 hardened, that is to say, which can be improved  
by a precipitation hardening and which is after  
such precipitation hardening stable against the  
high temperatures to which it had been subjected  
during the annealing treatment causing the pre-  
25 cipitation hardening. These alloys are first  
quenched for the purpose of attaining their high-  
est magnetic properties, and then annealed at  
elevated temperatures (up to about 700° C.). In  
consequence of this heat treatment they are  
30 completely stable to temperature changes up to  
the previous annealing temperature. After heat-  
ing to elevated temperatures they revert to their  
initial values on cooling. This property is fre-  
quently very desirable in the construction of  
35 machines, apparatus and measuring instruments.  
It could however, up to the present, not be at-

tained with the magnetic alloys hitherto usual.  
Such requirements are for example, made in the  
construction of temperature regulators, contacts,  
measuring instruments and the like.

By way of example an alloy may be mentioned, 30  
the main constituents of which are 15 per cent of  
tungsten and 30 per cent of cobalt, the remainder  
being iron. If such an alloy be quenched from  
1200° C. and be annealed for one hour at 700° C.  
there is thus obtained a coercive force of about 65  
85 gausses. The alloy thus treated can now be  
heated, to a temperature of about 700° C. with-  
out its magnetic hardness being decreased there-  
by. This process is generally known as "age  
hardening" or precipitation hardening. 70

I claim:—

1. A permanent magnet resistant to tempera-  
ture changes which comprises a ferromagnetic  
alloy magnetically stable against temperature  
changes up to about 700° C. 75

2. A permanent magnet resistant to tempera-  
ture changes which comprises a ferromagnetic  
alloy subjected to precipitation hardening, con-  
taining as main constituents, 15 per cent of  
tungsten and 30 per cent of cobalt and the re- 80  
mainder iron.

3. A method of preparing an alloy for perma-  
nent magnets, which consists in precipitation  
hardening of a ferromagnetic alloy by first  
quenching said alloy from a temperature of about 85  
1200° C. for the purpose of obtaining its highest  
magnetic properties, and then annealing the alloy  
at temperatures up to 700° C., said alloy contain-  
ing as main constituents approximately 15%  
tungsten, 30% cobalt and the remainder iron. 90

WERNER KÖSTER.

## DISCLAIMER

1,928,382.—Werner Köster, Dortmund, Germany. PERMANENT MAGNET. Patent  
dated September 26, 1933. Disclaimer filed August 2, 1938, by the assignee,  
Deutsche Edelstahlwerke A. G.

Hereby enters this disclaimer to claim 1 in said specification.  
[Official Gazette September 6, 1938.]

**DISCLAIMER**

1,928,382.—*Werner Köster*, Dortmund, Germany. PERMANENT MAGNET. Patent dated September 26, 1933. Disclaimer filed August 2, 1938, by the assignee, *Deutsche Edelstahlwerke A. G.*

Hereby enters this disclaimer to claim 1 in said specification.  
[*Official Gazette September 6, 1938.*]